

Oct. 18, 1955

P. D. WILLIAMS

2,721,155

METHOD OF CARBURIZING TUNGSTEN FILAMENTS

Original Filed Feb. 27, 1950



Fig. 1



Fig. 2



Fig. 3



Fig. 4



Fig. 5



Fig. 6



Fig. 7



INVENTOR.  
Paul D. Williams  
BY *Harold E. Long*

ATTORNEY

2,721,155

## METHOD OF CARBURIZING TUNGSTEN FILAMENTS

Paul D. Williams, Palo Alto, Calif., assignor to Eitel-McCullough, Inc., San Bruno, Calif., a corporation of California

Original application February 27, 1950, Serial No. 146,507, divided and this application August 27, 1951, Serial No. 243,889

3 Claims. (Cl. 148—13.1)

This is a division of my copending application Serial No. 146,507, filed February 27, 1950, now U. S. Patent 2,625,666.

My invention relates to filamentary cathodes for electron tubes, and more particularly to improvements in thoriated tungsten type filaments.

Thoriated tungsten wire comprising tungsten containing thorium oxide (thoria) is widely used in making filaments for electron discharge devices such as radio transmitting tubes. The practice is to form such filaments of solid thoriated tungsten wire, shaped as hairpins or other desired shapes, which filaments are mounted on a suitable stem structure. In order to improve the electron emission properties of the filament the thoriated tungsten wire is carburized to convert the outer portions of the wire to tungsten carbide, the practice being to heat the mounted filament in an atmosphere containing carbon, such as a hydrocarbon, to effect carburization.

The most serious disadvantage of such filaments is that they are brittle and fragile, due principally to the fact that a goodly portion of the solid cross-section of each filament wire is carburized. These fragile filaments constitute one of the weakest elements in the tube and are responsible for much loss due to breakage, both in commercial and military applications, particularly when the tube is subjected to shock and vibration.

The broad object of my invention is to improve the strength of thoriated tungsten filaments.

Another object is to achieve the improved strength without impairing the electron emission properties of the filament.

A further object is to provide a filament-making material which may be readily fabricated in the initial stage, and which is easily handled and processed during tube manufacture.

The invention possesses other objects and features of advantage, some of which, with the foregoing, will be set forth in the following description of my invention. It is to be understood that I do not limit myself to this disclosure of species of my invention as I may adopt variant embodiments thereof within the scope of the claims.

Referring to the drawing:

Figure 1 is an elevational view of a filament structure embodying my improved filaments.

Figures 2 and 3 are enlarged cross-sectional views of a filament before and after carburization; and

Figures 4 and 5 are side views of the same.

Figures 6 and 7 are cross-sectional views of modified type of filament before and after carburization; and

Figures 8 and 9 are side views of the same.

In terms of broad inclusion, my improved filament for electron tubes comprises a bundle of twisted strands of thoriated tungsten wire. In its preferred form the bundle is made up of several twisted wire ropes, each rope comprising twisted strands of the thoriated tungsten wire. Preferably only certain portions of the stranded filament are carburized to form a carburized zone running helical-

ly of the filament. To facilitate carburization of the filament, a carbon bearing thread is preferably intertwined with the wire, which thread is preferably wound helically of the filament axis. The filament material thus formed is suitably mounted on a supporting stem, after which the filament is heated to disintegrate the thread and carburize the wire.

In greater detail, and referring first to Figure 1 of the drawing, my improved filament for electron tubes is illustrated as a filamentary cathode structure comprising a plurality of parallel filaments 10. The structure shown has a glass stem 11 carrying a pair of metallic leads 12 and a central standard 13 sealed to a press 14 of the stem. Flexible extensions 16 on the leads serve to make connections with the base of the tube. A cup-shaped metal shield 17 fastened to standard 13 and embracing the press 14 serves to protect the glass stem.

In the filament structure illustrated, the filaments 10 are maintained under tension. The lower ends of certain of the filaments are welded to a fixed arcuate support 18 on one of the leads 12, and the lower ends of the remaining filaments are welded to a second, fixed arcuate support 18 on the other lead 12. All of the filaments are welded at the upper end to a circular support 19 slidable on the standard 13. By this arrangement the filament heating current passes up through half of the filaments and down through the other half. The filaments are tensioned by a coil spring 22 encircling standard 13 and interposed between a stop 23 and a compression sleeve 24 extending upwardly and bearing against a cup 26 under the slidable support 19.

The above described stem construction is merely for purposes of illustration, it being understood that other suitable filament supporting structures may be employed. The individual filaments 10 embodying my improvements each comprise a bundle of twisted strands of thoriated tungsten wire. In the form shown in Figures 2 to 5 the filament is made up of a uniform circular bundle of twisted strands 27. The strands 27 are of an ordinary commercial grade of thoriated tungsten wire, the size and number of strands depending upon the diameter of filament desired. The diameter of the individual strands is preferably quite small so that a relatively large number of strands are provided in the bundle, the multiplicity of small strands being partially responsible for the improved strength compared to the usual filament of solid cross-section. For example, I prefer to use 21 strands of .002 inch diameter wire to produce a filament having electron emission properties similar to a .010 inch diameter filament of solid cross-section. Filaments made up of strands of .001 inch diameter wire have been used, but wires of such small diameter are harder to handle in a twisting machine. The strands may be twisted together in any suitable type of twisting machine, a sufficient number of twists being provided to hold the strands together.

As above mentioned, the stranded character of the filament is partially responsible for the improved strength and pliability of the filament. Another very important factor, in combination with stranded feature, is the distribution of carbon in the final carburized product. The stranded filament is only partially carburized, preferably to provide a carburized zone running helically of the filament, so that a quantity of uncarburized strands are preserved to maintain the strength of the filament. Such distribution of carbon is conveniently accomplished by intertwisting with the strands 27 a carbon bearing thread 28. This may be an ordinary white cotton thread and may be impregnated with aquadag, if desired, to increase the carbon content. The thread is preferably incorporated so that it lies as a helix along the filament, ad-

jaacent the outer strands of wire in the bundle, as shown in Figures 2 and 4.

The wire so fabricated and including the thread may be produced in long lengths by the wire manufacturer and supplied on the spool to the tube industry, in the same manner that solid thoriated tungsten filament making wire is now supplied to the trade. At the tube plant the stranded filament material is cut to length and the filaments are mounted by welding or otherwise to the filament supporting in the usual manner. During this 10 mounting stage the stranded filaments have an advantage because they are more flexible and therefore more easily handled than filaments of solid cross section.

After mounting, the improved filaments are carburized by the simple expedient of heating the filaments in an oxygen free atmosphere, such as in hydrogen or in a vacuum, to a temperature sufficient to disintegrate the thread and carburize the wire. Heating the filaments to a temperature of about 2100° C. is adequate for this purpose. The thoriated tungsten strands adjacent the thread are thus carburized in a zone 29 running helically of the filament as indicated in Figures 3 and 5.

In order to obtain maximum strength I prefer to use a form of stranded filament shown in Figures 6 to 9 wherein the bundle is made up of several twisted ropes 31, each rope comprising twisted strands 32 of the thoriated tungsten wire. For example, I have had good results using three twisted ropes, each rope comprising seven twisted strands of .002 inch diameter wire, to produce a filament having electron emission properties similar to a .010 inch diameter filament of solid cross section. As seen in Figure 8, the strands 32 of a given rope preferably have tighter twists than the twists between the ropes 31. This provides an interlocking action where the strands bind together between the ropes.

In this case the carburizing thread 33 is preferably intertwined with the ropes 31 so that the thread follows the twist of the wire ropes as shown in Figures 6 and 8. After heating, a carburized zone 34 is provided running helically of the filament as indicated in Figures 7 and 9. It will be noted, because the individual strands have tighter twists than the ropes themselves, that the carburized zone runs crosswise of the separate wire strands. In other words, the carburized zone runs across the strands rather than following individual strands as in the case first described. Thus, a given strand is carburized in sections only, and, since the remaining sections of the strand are interlocked between the ropes, an additional measure of strength is obtained in the filament.

I have found that filaments made in accordance with my invention have good electron emission efficiency and filament life characteristics. I have also made extensive shock tests to compare the improved filaments with those commonly used in the art. These comparative tests were made with electron tubes having filament stem structures similar to that shown in Figure 1, the tubes being substantially the same except that in one case the

filaments were of the carburized stranded type shown in Figures 7 and 9, and in the other case were ordinary carburized solid wire filaments. A standard impact machine for electron tubes was employed in making the 5 shock tests. The results showed that the ordinary filaments broke at an average of about 100 G. shock acceleration, while the improved filaments broke at an average of over 400 G., constituting an improvement of better than 300% in shock resistance.

Instead of employing a thread to carburize the filament, my improved stranded type filament may be carburized in the ordinary manner by heating it in a hydrocarbon atmosphere. For example, the stem shown in Figure 1, with the stranded filaments mounted in place, 15 may be positioned in a bell jar containing a hydrocarbon atmosphere, such as benzene, and the filaments heated sufficiently to absorb carbon from the atmosphere. In this case the outer strands of each filament are uniformly carburized, leaving the strands in the core portions of the filament uncarburized. This type of carburized stranded filament does not have the maximum strength, 20 but is still superior to an ordinary filament of solid cross section carburized in the same manner. Compared to ordinary filaments breaking at an average of about 100 G. 25 shock acceleration, the last mentioned stranded filaments broke at an average of about 200 G., showing an improvement of about 100% in shock resistance.

I claim:

1. The method of making a filamentary cathode, which 30 comprises mounting a filament containing a thread of carbon bearing material and thoriated tungsten wire, said thread engaging a selected portion only of the surface of the wire, and then heating the filament to a temperature of about 2100° C. to disintegrate the thread and carburize the selected portion of the wire.
2. The method of making a filamentary cathode, which 35 comprises mounting a filament containing a thread of carbon bearing material intertwined with strands of thoriated tungsten wire, said thread engaging a selected portion only of the surface of the wire, and then heating the filament to a temperature of about 2100° C. to disintegrate the thread and carburize the selected portion of the wire.
3. The method of making a filamentary cathode, which 40 comprises mounting a filament containing carbon bearing 45 thread helically wound with strands of thoriated tungsten wire, said thread engaging a selected portion only of the surface of the wire, and then heating the filament to a temperature of about 2100° C. to disintegrate the thread and carburize the selected portion of the wire.

#### References Cited in the file of this patent

#### UNITED STATES PATENTS

- |    |           |                 |               |
|----|-----------|-----------------|---------------|
| 55 | 376,194   | Harvey          | Jan. 10, 1888 |
|    | 2,397,553 | Chevigny        | Apr. 2, 1946  |
|    | 2,495,167 | Horstman et al. | Jan. 17, 1950 |